

Aug. 27, 1957

H. G. SCHURECHT

2,804,392

SPARK PLUG INSULATORS CONTAINING ZnO

Filed April 25, 1952

4 Sheets-Sheet 1



FIG. 1.



INVENTOR  
Harry G. Schurecht  
BY  
Owen & Owen

ATTORNEYS

Aug. 27, 1957

H. G. SCHURECHT

2,804,392

SPARK PLUG INSULATORS CONTAINING  $ZnO$

Filed April 25, 1952

4 Sheets-Sheet 2



FIG. 3.



FIG. 4.

INVENTOR  
Harry G. Schurecht  
BY Owen & Owen

ATTORNEY

Aug. 27, 1957

H. G. SCHURECHT

2,804,392

SPARK PLUG INSULATORS CONTAINING  $ZnO$

Filed April 25, 1952

4 Sheets-Sheet 3



INVENTOR  
Harry G. Schurecht  
BY *Owen & Owen*  
ATTORNEYS

Aug. 27, 1957

H. G. SCHURECHT

2,804,392

SPARK PLUG INSULATORS CONTAINING  $ZnO$

Filed April 25, 1952

4 Sheets-Sheet 4



FIG. 7.



FIG. 8.

INVENTOR  
Harry G. Schurecht  
BY  
Owen & Owen  
ATTORNEYS

1

2,804,392

## SPARK PLUG INSULATORS CONTAINING ZnO

Harry G. Schurecht, Detroit, Mich., assignor to Champion Spark Plug Company, Toledo, Ohio, a corporation of Delaware

Application April 25, 1952, Serial No. 284,470

13 Claims. (Cl. 106—46)

This invention relates to electrical insulators which contain zinc oxide, and which are suitable for spark plugs and for similar uses.

Zinc oxide has heretofore been suggested as a flux for use with high alumina spark plug insulator bodies, as an alternative to alkaline earth compounds frequently used. Relatively satisfactory high alumina insulators can be produced using zinc oxide in the proportions in which fluxes are ordinarily employed. When the proportion of zinc oxide is increased above that usually employed as a flux, however, the hot dielectric properties of the resulting insulators are so poor as to be unsatisfactory for any spark plug use. For example, an insulator made from zinc oxide and alumina, in the proportions of about 25 mol percent and about 75 mol percent, respectively, has an electrical resistance of substantially less than 1 megohm at 1350° F., measured as described in Example 1 hereof, and it is generally accepted that spark plug insulators for high compression engines must have a minimum resistance of at least 1 megohm at 1350° F. to be satisfactory. Increasing the proportion of zinc oxide above 25 percent further decreases the electrical resistance of insulators containing it.

The present invention is based upon the discovery that electrical insulators meeting the exacting requirements for use as spark plug insulators in high compression engines burning leaded fuel can be produced from alumina and zinc oxide when the latter is present in higher proportions than heretofore employed, and that such spark plug insulators can also be produced from blends in certain proportions of zinc oxide with alumina, beryllia, magnesia, oxides of cerium, tin, zirconium, titanium, calcium, strontium, barium, and boron.

In the drawings,

Fig. 1 is a triaxial diagram showing the proportions in mol percentages in which alumina, beryllia, and ZnO can be used to produce electrical insulators of the invention;

Fig. 2 is a triaxial diagram showing the proportions in mol percentages in which magnesia, beryllia, and ZnO can be used to produce electrical insulators of the invention;

Fig. 3 is a triaxial diagram showing the proportions in

2

mol percentages in which alumina, magnesia, and ZnO can be used to produce electrical insulators of the invention;

Fig. 4 is a regular tetrahedron showing the proportions in mol percentages in which alumina, beryllia, magnesia, and ZnO can be combined to produce electrical insulators of the invention;

Fig. 5 is another view of the tetrahedron shown in Fig. 4;

Fig. 6 is a combined view of Figs. 1, 2, and 3, on a reduced scale, illustrating the way these three figures are combined to produce Figs. 4 and 5;

Fig. 7 is a reproduction of Fig. 4 with lines added thereto to represent planes which identify preferred compositions; and

Fig. 8 is a reproduction of Fig. 4 with other lines added thereto to represent different planes which represent other preferred compositions.

According to the invention, a sintered ceramic electrical insulator suitable for spark plug and similar uses is provided. The electrical insulator shows, by chemical analysis, at least 60 percent by weight of a major component having a composition represented by the portion of Figs. 4 and 5 within the shaded planes, and from a trace to 40 percent by weight of a minor component. The minor component consists essentially of at least one modifying ingredient that is an oxide of one of the following metals: calcium, strontium, barium, boron, titanium, zirconium, cerium and tin. The insulator contains, from the minor component, not over 20 percent by weight of oxides of calcium, strontium, and barium, not over 5 percent by weight of an oxide of boron, and not over 20 percent by weight of oxides of titanium, zirconium, cerium and tin. The sum of the mols of oxides of titanium, zirconium, cerium, and tin is not more than half the sum of the mols of alumina and magnesia plus one-twentieth the mols of beryllia.

Referring now more particularly to the drawings, the shaded portion of Fig. 1, which represents compositions in mol percentages, shows the proportions in which alumina, beryllia, and zinc oxide can be combined prior to firing to produce electrical insulators having sufficiently high resistance at elevated temperatures, and sufficiently high thermal conductivity, for use as spark plug insulators. It will be observed that this shaded area may be designated 11—13—14—19—20—16—11. Insulators produced by firing bodies of compositions represented by the upper portion of this shaded area, 14—19—20—14, have extremely high heat conductivities, and are, for this reason, preferred spark plug insulators. Electrical insulators produced by firing compositions represented by the area between the lines 41—42 and 45—46 have extremely high electrical resistance at elevated temperatures, and, therefore, also constitute preferred compositions. Maximum thermal conductivities are obtained from composition represented along the line 15—22.

50

55

The compositions represented by the several points of Fig. 1 are shown in Table A, below:

TABLE A

| Point | Mol Percent |                                |        |
|-------|-------------|--------------------------------|--------|
|       | BeO         | Al <sub>2</sub> O <sub>3</sub> | ZnO    |
| 11    | 0           | 50                             | 50     |
| 12    | 0           | 33 1/3                         | 66 2/3 |
| 13    | 0           | 20                             | 80     |
| 14    | 80          | 0                              | 20     |
| 15    | 92.9        | 0                              | 7.1    |
| 16    | 20          | 60                             | 20     |
| 19    | 99.67       | 0                              | 0.33   |
| 20    | 79.67       | 20                             | 0.33   |
| 22    | 94.93       | 4.74                           | 0.33   |
| 41    | 97.9        | 0                              | 2.1    |
| 42    | 0           | 33 1/3                         | 66 2/3 |
| 45    | 87.9        | 0                              | 12 1/3 |
| 46    | 0           | 28 1/3                         | 71 2/3 |
| A     | 0           | 75                             | 25     |
| B     | 16 2/3      | 83 1/3                         | 0      |
| C     | 63.2        | 36.8                           | 0      |
| D     | 72.7        | 27.3                           | 0      |

Referring now to Fig. 2, electrical insulators produced by firing compositions represented by the area 14—19—24—27—14 have been found to be satisfactory for spark plug uses. Insulators produced by firing compositions represented by the area 14—19—28—14 are preferred because they have especially high thermal conductivities, and insulators produced by firing compositions represented by the area between the lines 40—41 and 44—45 are preferred because they have especially high electrical resistance at elevated temperatures. Maximum thermal conductivities are obtained from compositions represented along the line 15—26.

The compositions represented by the several points of Fig. 2 which are not given in Table A are shown in Table B, below:

TABLE B

| Point | Mol Percent |       |      |
|-------|-------------|-------|------|
|       | BeO         | MgO   | ZnO  |
| 24    | 0           | 99.67 | 0.33 |
| 25    | 0           | 92.6  | 7.4  |
| 26    | 90.61       | 9.06  | 0.33 |
| 27    | 0           | 60    | 40   |
| 28    | 62.29       | 37.38 | 0.33 |
| 40    | 0           | 97.6  | 2.4  |
| 44    | 0           | 87.6  | 12.4 |

Referring now to Fig. 3, the shaded area thereof, designated 11—13—27—24—17—11, represents compositions of alumina, magnesia, and zinc oxide which can be fired to produce electrical insulators having properties that make them suitable for spark plug and similar uses. The area between the lines 40—42 and 44—46 represents compositions which, when fired, have especially high electrical resistance at elevated temperatures. Point 17 represents a composition containing 60 mol percent of Al<sub>2</sub>O<sub>3</sub>, 20 mol percent of MgO, and 20 mol percent of ZnO.

Figs. 4 and 5 are two views of a tetrahedron representing the proportions of magnesia, beryllia, alumina, and zinc oxide operable for the production of electrical insulators of the invention. Fig. 5 shows the tetrahedron rotated counter clockwise 120° above a vertical axis through the upper or BeO vertex from the position shown in Fig. 4. In Fig. 4, the faces of the tetrahedron representing ternary mixtures of Al<sub>2</sub>O<sub>3</sub>, BeO, and ZnO (Fig. 1), and MgO, BeO, and ZnO (Fig. 2) are visible. A third boundary of the operable proportions faces the observer, but is hidden by the two faces of the tetrahedron; this surface is shaded with dotted lines, and is designated 13—14—27—13. Operable compositions containing alumina, magnesia, and ZnO are also represented in Fig. 4

and lie within the area 11—13—27—24—17—11. This area is not shaded in Figs. 4 and 5 because shade lines would unnecessarily complicate the figures, and would make comprehension difficult. From the angle at which

5 the tetrahedron of Fig. 5 is viewed the remaining surfaces which bound the operable area can be seen readily. These surfaces are as follows: 11—16—17—11; 24—17—16—24; 24—16—20—24; and 24—20—19—24. All of these identified areas are invisible, and are shaded with 10 dotted lines, because they lie behind the faces of the tetrahedron. The surface representing ternary mixtures of BeO, Al<sub>2</sub>O<sub>3</sub>, and ZnO (Fig. 1) is visible in Fig. 5. The other two surfaces bounding the operable area (24—27—14—19—24, Fig. 2, and 11—13—27—24—17—11, Fig. 15 3) can also be identified in Fig. 5.

Compositions represented by the portion of Fig. 4 enclosed by a plane through the points 14, 20, and 28, a plane through 14, 20, and 19, a plane through 14, 19, and 28, and a fourth plane through 19, 20, and 28 are preferred 20 because electrical insulators fired therefrom have especially high thermal conductivities. Compositions represented by the portion of Fig. 4 between a plane through the points 40, 41, and 42 and a second plane through the 25 points 44, 45, and 46 are also preferred because insulators therefrom have especially high electrical resistance at elevated temperatures.

Still another group of preferred compositions represented on Fig. 7 lies between a plane through the points 25, 19, 11 and a second plane through the points 25, 14 and 13.

Fig. 6 shows the tetrahedron of Figs. 4 and 5 with its three faces which meet at the BeO vertex rotated about their respective base lines opposite the BeO vertex into the plane of the base of the tetrahedron. It will be apparent from observation of Fig. 6 that Figs. 1, 2, and 3 are represented therein; from this it is apparent that the tetrahedron of Figs. 4 and 5 is derived from Figs. 1, 2, and 3. It is known that the compositions which result from mixing, in all proportions, two mixtures represented by two 35 points on a triaxial diagram are represented by a straight line joining those two points. Similarly, the compositions which result from mixing, in all proportions, two binary, ternary or quaternary mixtures represented on a regular tetrahedron, are represented by a straight line joining 40 those two points. It follows, therefore, that the plane in Fig. 4 through the points 13, 14, and 27, for example, represents the compositions of mixtures, in all proportions, of a binary blend of alumina and zinc oxide represented by the point 13, a binary mixture of beryllia and 45 zinc oxide represented by the point 14, and a binary mixture of magnesia and zinc oxide represented by the point 27. From the foregoing it follows, also, that the portions of Figs. 4 and 5 bounded by the shaded planes represent mixtures in all proportions of compositions represented 50 by the shaded areas of Figs. 1, 2, and 3.

It has been found that, within the limits of the compositions of MgO, BeO, ZnO and Al<sub>2</sub>O<sub>3</sub> claimed herein, if two bodies of different composition each produce insulators satisfactory for spark plug uses, then insulators produced from compositions that may be considered to be blends of the two compositions will also produce insulators satisfactory for spark plug uses. Bodies 31, 32, and 60 36 from Table II, below, demonstrate this principle, as do bodies 1, 4, 5, 36, 38, 40, 41, 43, 44, and 45, from Tables I and II, below.

The suitability for use in the manufacture of electrical insulators for spark plug purposes of various compositions within the portion of Figs. 4 and 5 bounded by the shaded planes, and containing additives or modifying oxides 70 within the proportions stated above, was demonstrated by preparing several insulators, and testing the properties of each. Compositions and properties for various insulators within the scope of the claims are given in the following examples, which are to be construed as illustrative only, and not as limiting the invention.

Sintered ceramic electrical insulators were prepared from various compositions including alumina, beryllia, and zinc oxide, plus minor amounts of an oxide of calcium, strontium, or barium introduced incidentally in the course of processing. In all cases, a blend of at least two of the three named ingredients was wet milled to substantial uniformity (usually for 18 hours), was then dried and mixed with 4 percent of paraffin wax, based upon the weight of dry ingredients, dissolved in carbon tetrachloride. The wax was thoroughly mixed with the dry ingredients, and the carbon tetrachloride volatilized, leaving the wax uniformly dispersed throughout the com-

mines porosity, strength and other properties. This was measured by a standard dye test. In the tables herein, the abbreviation "Mat." is used to indicate that the body was matured and completely satisfactory in this respect; 5 "O. B." to indicate that it was overburned; "U. F." that it was underfired; and "S" preceding either "U. F." or "O. B." that underfiring or overburning was slight. In general, an overburned or underfired body can be corrected by varying the flux content or the firing tempera- 10 ture.

Typical test results for bodies produced from two or more of the three named ingredients are presented in Table I. below:

- TABLE I

| Body No. | Mol Percent |                                |      | Dye Test |         | Electrical Resistance (Megohms) at 1,350° F. |         | Thermal Diffusivity, Seconds |         |
|----------|-------------|--------------------------------|------|----------|---------|----------------------------------------------|---------|------------------------------|---------|
|          | BeO         | Al <sub>2</sub> O <sub>3</sub> | ZnO  | Cone 16  | Cone 31 | Cone 16                                      | Cone 31 | Cone 16                      | Cone 31 |
| 1        | 84.4        | 6.9                            | 8.7  | —        | —       | 100+                                         | —       | 9.20                         | —       |
| 2        | 47.4        | 23.3                           | 29.2 | —        | —       | 100+                                         | —       | 17.40                        | —       |
| 3        | 71.5        | 17.5                           | 11.0 | U. F.    | O. F.   | 12                                           | 100+    | 18.5                         | 11.8    |
| 4        | 69.7        | 8.6                            | 21.5 | Mat.     | O. F.   | 50                                           | 60      | 8.5                          | 11.1    |
| 5        | 48.8        | 36.0                           | 15.1 | U. F.    | U. F.   | 6                                            | 100+    | 26.9                         | 17.0    |
| 6        | —           | 44.4                           | 55.6 | U. F.    | U. F.   | 100+                                         | 100+    | 24.0                         | —       |
| 7        | —           | 39.5                           | 60.5 | S. U. F. | O. F.   | 95                                           | 100+    | 24.8                         | 24.9    |
| 8        | —           | 34.6                           | 65.4 | S. U. F. | O. F.   | 100+                                         | —       | 20.9                         | 23.8    |
| 9        | —           | 34.9                           | 64.1 | —        | —       | 100+                                         | —       | 31.4                         | —       |
| 10       | 92.5        | —                              | 7.5  | Mat.     | O. F.   | 75                                           | —       | 5.3                          | 8.3     |

position. Test cylinders, about  $\frac{1}{2}$  inch in diameter and approximately  $\frac{1}{2}$  inch in length, were then pressed from the mixed composition using a total pressure of ten thousand pounds. These cylinders were then fired to Cone 16 or to Cone 31. The bodies so prepared were tested to determine their suitability for use as spark plug insulators. The electrical resistance of the  $\frac{1}{2}$  inch cylinder was determined at  $1350^{\circ}$  F. Although the resistance required of insulators for spark plugs depends to a certain extent upon the design of the plug, the minimum acceptable value should be at least 1 megohm at  $1350^{\circ}$  F. for such cylinders. Another standard test was conducted to compare the thermal diffusivities of insulators produced from the different compositions; the test

If, for purposes of comparison, but not in accordance with the invention, insulators are produced as described above from compositions containing 83.4 mol percent of ZnO, 45.5 mol per cent of ZnO, and 23.8 mol percent of ZnO, balance alumina, in each instance the electrical resistance at 1350° F. is found to be less than 1 megohm. Such insulators, accordingly, are not suited for spark plug uses. Similarly, insulators containing more than 16½ mol percent, and up to 72.7 mol percent, of beryllia, balance alumina, are relatively unsatisfactory for spark plug purposes.

45 For purposes of comparison, the characteristics of substantially pure zinc oxide insulators, prepared as described above, are also presented in Table C, below:

TABLE C

| Body No. | Mol<br>Percent<br>ZnO | Additives Grams per<br>1,000 Grams ZnO |       |                | Dye<br>Test<br>Cone<br>16 | Electrical<br>Resistance (Megohms)<br>of $\frac{1}{2}$ cylinder |           | Thermal<br>Diffu-<br>sivity,<br>Seconds |
|----------|-----------------------|----------------------------------------|-------|----------------|---------------------------|-----------------------------------------------------------------|-----------|-----------------------------------------|
|          |                       | Whiting                                | Talc  | Bent-<br>onite |                           | 900° F.                                                         | 1,000° F. |                                         |
| I        | 100                   | -----                                  | ----- | -----          | Mat                       | 0.1                                                             | -----     | 15.9                                    |
| II       | 100                   | 15.5                                   | ----- | -----          | Mat                       | 0.3                                                             | 0.05      | 13.8                                    |
| III      | 100                   | 15.5                                   | ----- | 15.5           | Mat                       | 0.02                                                            | -----     | 15.0                                    |
| IV       | 100                   | 15.5                                   | 20.8  | 15.5           | Mat                       | 0.02                                                            | -----     | 15.0                                    |
| V        | 100                   | 31.5                                   | 25.9  | 15.5           | Mat                       | 23.0                                                            | 0.01      | 17.7                                    |

involved placing a crystal of citric acid on one end of the sintered  $\frac{1}{2}$ -inch cylinder, and immersing the other end of the cylinder in a  $600^{\circ}$  F. metal bath to a depth of  $\frac{1}{8}$  inch. The number of seconds required for heat conducted through the insulator to melt the citric acid crystal, which melts at  $307.4^{\circ}$  F., is reported in the tables herein as "thermal diffusivity," and is an inverse function of thermal conductivity. To be satisfactory for spark plug use an insulator should have a thermal diffusivity, so measured, not greater than 50 seconds, and preferably not greater than 40 seconds. The adequacy of the firing under a set of standard conditions is also an important characteristic of a ceramic composition since it deter-

*Example 2*

65 Table II, below, presents typical test results obtained  
with bodies containing varying proportions of  $\text{Al}_2\text{O}_3$ ,  
 $\text{BeO}$ ,  $\text{ZnO}$ , and various additives, and demonstrates, in  
conjunction with Table I, the general proposition that  
where a body has been produced containing two or more  
70 of the principal ingredients,  $\text{Al}_2\text{O}_3$ ,  $\text{BeO}$ ,  $\text{ZnO}$ , and  $\text{MgO}$ ,  
a satisfactory body can be produced from these ingre-  
dients in the same proportions, but containing small  
amounts of the additives or modifying ingredients  
claimed herein. In all instances, the bodies reported in  
75 Table II were produced in the same way as the bodies  
reported in Table I.

TABLE II

| Body No. | Mol Percent |                                |      | Additives, Grams per 1,000 grams BeO, Al <sub>2</sub> O <sub>3</sub> and ZnO | Electrical Resistance (Megohms) at 1,350° F. |         | Thermal Diffusivity, Seconds |         | Dye Test |          |
|----------|-------------|--------------------------------|------|------------------------------------------------------------------------------|----------------------------------------------|---------|------------------------------|---------|----------|----------|
|          | BeO         | Al <sub>2</sub> O <sub>3</sub> | ZnO  |                                                                              | Cone 16                                      | Cone 31 | Cone 16                      | Cone 31 | Cone 16  | Cone 31  |
| 11       |             | 21.6                           | 78.4 |                                                                              | 15                                           | 90      | 44.8                         |         | U. F.    |          |
| 12       | 92.5        |                                | 7.5  | Whiting 15.5 grams                                                           | 100+                                         | 100+    | 5.8                          | 8.7     | Mat.     | Mat.     |
| 13       | 92.5        |                                | 7.5  | 15.5 grams each of Whiting and Bentonite.                                    | 100+                                         | 95      | 5.6                          | 6.6     | S. U. F. | Mat.     |
| 14       | 92.5        |                                | 7.5  | (*)                                                                          | 90                                           | 100+    | 5.9                          | 8.0     | Mat.     | Mat.     |
| 15       | 86.0        |                                | 14.0 | (*)                                                                          | 6                                            | 9       | 6.7                          | 8.7     | S. U. F. | Mat.     |
| 16       | 83.0        |                                | 17.0 | (*)                                                                          | 8                                            |         | 7.0                          | 8.9     | Mat.     | Mat.     |
| 17       | 92.5        |                                | 7.5  | 15.5 grams Bentonite                                                         |                                              | 1.5     | 11                           | 5.7     | 9.2      | Mat.     |
|          |             |                                |      | 25.9 grams ZrO <sub>2</sub>                                                  |                                              |         |                              |         |          | Mat.     |
|          |             |                                |      | 31.0 grams Whiting                                                           |                                              |         |                              |         |          |          |
| 18       | 98.7        |                                | 1.3  | 64.0 A*                                                                      | 100+                                         | 100+    | 8.0                          |         | U. F.    | Mat.     |
| 19       | 97.0        |                                | 3.0  | 136.8 A*                                                                     | 55                                           | 58      | 6.4                          |         | U. F.    | S. U. F. |
| 20       | 95.0        |                                | 5.0  | 219.0 A*                                                                     | 55                                           | 55      | 11.7                         |         | U. F.    | S. U. F. |
| 21       | 98.8        |                                | 1.2  | 69.4 B*                                                                      | 100+                                         | 100+    | 6.7                          |         | U. F.    | Mat.     |
| 22       | 97.4        |                                | 2.6  | 149.3 B*                                                                     | 100+                                         | 100+    | 6.5                          |         | S. U. F. | Mat.     |
| 23       | 95.6        |                                | 4.4  | 241.0 B*                                                                     | 32                                           | 33      | 6.6                          |         | S. U. F. | Mat.     |
| 24       | 98.9        |                                | 1.1  | 72.8 C*                                                                      | 100+                                         |         | 6.0                          |         | Mat.     |          |
| 25       | 97.6        |                                | 2.4  | 157.0 C*                                                                     | 72                                           |         | 6.5                          |         | Mat.     |          |
| 26       | 96.0        |                                | 4.0  | 250.0 C*                                                                     | 30                                           |         | 6.7                          |         | Mat.     |          |
| 27       | 98.4        |                                | 1.6  | 52.2 D*                                                                      | 90                                           |         | 6.9                          |         | Mat.     |          |
| 28       | 96.3        |                                | 3.7  | 110.0 D*                                                                     | 28                                           |         | 6.9                          |         | Mat.     |          |
| 29       | 93.8        |                                | 6.2  | 166.5 D*                                                                     | 3                                            |         | 7.2                          |         | Mat.     |          |
| 30       | 98.0        |                                | 2.0  | (**)                                                                         | 38                                           |         | 6.3                          |         | Mat.     |          |
| 31       | 22.6        | 54.8                           | 22.5 | (**)                                                                         | 50                                           | 100+    | 29.7                         |         | U. F.    |          |
| 32       | 28.6        | 43.5                           | 27.7 | (**)                                                                         | 90                                           | 100+    | 24.1                         |         | U. F.    |          |
| 33       | 28.8        | 35.6                           | 35.6 | (**)                                                                         | 100+                                         | 100+    |                              | 15.8    | U. F.    |          |
| 34       | 33.2        | 34.6                           | 32.1 | (**)                                                                         | 95                                           | 100+    | 23.8                         |         | U. F.    |          |
| 35       | 37.1        | 25.8                           | 27.0 | (**)                                                                         | 100+                                         |         | 17.7                         |         | Mat.     |          |
| 36       | 41.0        | 18.2                           | 40.7 | (**)                                                                         | 90                                           |         | 16.8                         |         | Mat.     |          |
| 37       | 47.7        | 26.1                           | 26.1 | (**)                                                                         | 92.5                                         | 100+    | 19.2                         | 13.8    | U. F.    | Mat.     |
| 38       | 53.9        | 20.0                           | 26.0 | (**)                                                                         | 100+                                         | 100+    |                              | 15.9    | U. F.    | Mat.     |
| 39       | 61.0        | 19.4                           | 19.4 | (**)                                                                         | 72.3                                         | 100+    | 16.7                         | 9.4     | U. F.    | Mat.     |
| 40       | 72.3        | 9.9                            | 16.9 | (**)                                                                         | 100+                                         |         | 9.0                          | 8.5     | Mat.     | Mat.     |
| 41       | 76.7        | 15.3                           | 8.1  | (**)                                                                         | 95                                           | 85      |                              | 10.5    | U. F.    | Mat.     |
| 42       | 84.5        | 7.7                            | 7.7  | (**)                                                                         | 92.5                                         | 100+    | 10.4                         | 5.8     | U. F.    | Mat.     |
| 43       | 89.5        | 5.3                            | 5.3  | (**)                                                                         | 66.0                                         | 100+    |                              | 9.4     | 5.8      | U. F.    |
| 44       | 93.6        | 3.2                            | 3.2  | (**)                                                                         | 92.5                                         | 100+    | 8.33                         | 6.0     | U. F.    | Mat.     |
| 45       | 96.9        | 1.5                            | 1.5  | (**)                                                                         | 70.0                                         | 100+    |                              | 5.3     | U. F.    | Mat.     |

\*Indicates that additives consisting of 15.5 grams whiting, 20.7 grams of talc, and 15.5 grams of bentonite were mixed with 1,000 grams of the indicated composition. When a number is followed by a letter and an asterisk, the number indicates the number of grams of a modifying ingredient referred to by the letter mixed with 1,000 grams of the composition, and the asterisk indicates whiting, talc, and bentonite in the quantities stated above. A refers to ZrO<sub>2</sub>; B to SnO<sub>2</sub>; C to CeO<sub>2</sub>; and D to TiO<sub>2</sub>.

\*\*Body 30 contained 104 grams of whiting and 21.6 grams of talc per 1,000 grams of BeO and ZnO.

### Example 3

In addition to the representative bodies in Tables I and II wherein alumina was employed, other bodies containing at least two of the ingredients ZnO, BeO, and MgO have been produced to demonstrate the operability of

40 bodies fired from such compositions in the proportions claimed herein. Representative examples thereof are presented in Table III, below. In all instances, the insulators were prepared in the manner described in Example 1.

TABLE III

| Body No. | Mol Percent |      |      | Additives, Grams per 1,000 grams BeO, MgO, and ZnO            | Electrical Resistance (Megohms) at 1,350° F. |         | Thermal Diffusivity, Seconds |         | Dye Test |         |  |
|----------|-------------|------|------|---------------------------------------------------------------|----------------------------------------------|---------|------------------------------|---------|----------|---------|--|
|          | BeO         | MgO  | ZnO  |                                                               | Cone 16                                      |         | Cone 16                      | Cone 31 | Cone 16  | Cone 31 |  |
|          |             |      |      |                                                               | Cone 16                                      | Cone 31 |                              |         |          |         |  |
| 46       | 95.5        | 2.2  | 2.2  | (*)                                                           | 100+                                         |         | 6.4                          | 5.9     | S. U. F. | Mat.    |  |
| 47       | 90.5        | 4.7  | 4.7  | (*)                                                           | 87                                           |         | 6.8                          | 5.5     | S. U. F. | Mat.    |  |
| 48       | 21.8        | 47.3 | 21.0 | (*)                                                           | 68                                           |         | 30.9                         |         | Mat.     |         |  |
| 49       | 18.3        | 56.5 | 24.2 | (*)                                                           | 9                                            |         | 22.9                         | 23.4    | Mat.     | Mat.    |  |
| 50       | 17.2        | 66.2 | 16.6 | (*)                                                           | 87                                           |         | 29.8                         |         | Mat.     |         |  |
| 51       | 12.3        | 75.4 | 12.2 | (*)                                                           | 100+                                         |         | 29.2                         |         | Mat.     |         |  |
| 52       | 8.0         | 83.9 | 7.9  | (*)                                                           | 100+                                         |         | 23.7                         |         | Mat.     |         |  |
| 53       | 3.9         | 92.0 | 3.9  | (*)                                                           | 33                                           |         | 22.6                         |         | Mat.     |         |  |
| 54       |             | 97.9 | 2.1  | 64.0 A*                                                       | 68                                           |         | 24.4                         |         | Mat.     |         |  |
| 55       |             | 95.3 | 4.7  | 136.8 A*                                                      | 40                                           |         | 30.8                         |         | Mat.     |         |  |
| 56       |             | 92.2 | 7.8  | 219.0 A*                                                      | 60                                           |         | 33.3                         |         | Mat.     |         |  |
| 57       |             | 98.1 | 1.9  | 69.4 B*                                                       | 100+                                         |         | 28.8                         |         | S. U. F. |         |  |
| 58       |             | 95.8 | 4.2  | 149.3 B*                                                      | 100+                                         |         | 30.5                         |         | S. U. F. |         |  |
| 59       |             | 93.0 | 7.0  | 241.0 B*                                                      | 95                                           |         | 36.4                         |         | S. U. F. |         |  |
| 60       |             | 96.2 | 3.8  | 187.0 C*                                                      | 100+                                         |         | 27.4                         |         | Mat.     |         |  |
| 61       |             | 93.7 | 6.3  | 256.0 C*                                                      | 87                                           |         | 27.8                         |         | Mat.     |         |  |
| 62       |             | 96.8 | 3.2  | 104 gms. Whiting<br>(16.2 gms. Bentonite<br>218 gms. Whiting) | 50                                           |         | 23.8                         |         | Mat.     |         |  |
| 63       |             | 93.2 | 6.8  | 22.5 gms. Talc<br>16.9 gms. Bentonite                         | 62                                           |         | 18.3                         |         | Mat.     |         |  |
| 64       |             | 80.5 | 11.3 | 8.2                                                           |                                              |         |                              | 8.05    |          |         |  |
| 65       |             | 63.2 | 27.1 | 9.7                                                           |                                              |         |                              | 11.10   |          |         |  |
| 66**     |             | 40.5 | 34.6 | 24.9                                                          | 100+ at 1,100° F.                            |         |                              | 17.28   |          |         |  |

\*Indicates that additives consisting of 15.5 grams whiting, 20.7 grams of talc, and 15.5 grams of bentonite were mixed with 1,000 grams of the indicated composition. When a number is followed by a letter and an asterisk the number indicates the number of grams of a modifying ingredient referred to by the letter mixed with 1,000 grams of the composition, and the asterisk indicates whiting, talc, and bentonite in the quantities stated above. A refers to ZrO<sub>2</sub>; B to SnO<sub>2</sub>; and C to CeO<sub>2</sub>.

\*\*Body 66 was not tested above 1,100° F.

## Example 4

Examples of bodies containing  $\text{Al}_2\text{O}_3$ ,  $\text{MgO}$ , and  $\text{ZnO}$  are presented in Table IV, below. In each instance the bodies were prepared by a procedure identical with that described in Example 1.

TABLE IV

| Body No. | Mol Percent             |              |              | Additives, Grams per 1,000 grams $\text{Al}_2\text{O}_3$ , $\text{MgO}$ and $\text{ZnO}$ | Electrical Resistance (Megohms) at 1,350° F. | Thermal Diffusivity, Seconds |         | Dye Test, Cone 16 |
|----------|-------------------------|--------------|--------------|------------------------------------------------------------------------------------------|----------------------------------------------|------------------------------|---------|-------------------|
|          | $\text{Al}_2\text{O}_3$ | $\text{MgO}$ | $\text{ZnO}$ |                                                                                          |                                              | Cone 16                      | Cone 31 |                   |
| 67       | 2.3                     | 95.1         | 2.3          | (*)                                                                                      | 100+                                         | 23.7                         | 14.8    | Mat.              |
| 68       | 4.9                     | 90.0         | 4.9          | (*)                                                                                      | 100+                                         | 98                           | 27.3    | Mat.              |
| 69       | 7.9                     | 84.1         | 7.9          | (*)                                                                                      | 100+                                         | 100+                         | 31.3    | 20.2 Mat.         |
| 70       | 11.4                    | 77.4         | 11.3         | (*)                                                                                      | 100+                                         | 98                           | 33.4    | 22.3 Mat.         |
| 71       | 14.3                    | 70.3         | 15.4         | (*)                                                                                      | 100+                                         | -----                        | 36.5    | S. U. F.          |
| 72       | 19.9                    | 60.2         | 19.9         | (*)                                                                                      | 92                                           | 100+                         | 40.8    | S. U. F.          |
| 73       | 27.9                    | 47.6         | 24.4         | (*)                                                                                      | 38                                           | 100+                         | 28.1    | S. U. F.          |
| 74       | 34.5                    | 34.8         | 30.7         | (*)                                                                                      | 50                                           | 85                           | 29.8    | S. U. F.          |
| 75       | 42.5                    | 19.3         | 38.2         | (*)                                                                                      | 100+                                         | -----                        | 29.4    | Mat.              |
| 76       | 58.1                    | 20.9         | 20.9         | (*)                                                                                      | 19                                           | 100+                         | 47.8    | U. F.             |
| 77       | 47.2                    | 26.4         | 26.4         | (*)                                                                                      | 95                                           | 100+                         | 43.9    | 23.1 U. F.        |
| 78       | 37.2                    | 31.3         | 31.3         | (*)                                                                                      | 100+                                         | -----                        | 30.7    | 24.5 Mat.         |

\*Indicates that the additives consisted of 15.5 grams of whiting, 20.7 grams of talc, and 15.5 grams of bentonite per 1,000 grams of  $\text{Al}_2\text{O}_3$ ,  $\text{MgO}$  and  $\text{ZnO}$ .

## Example 5

Insulators were prepared containing various proportions of  $\text{BeO}$ ,  $\text{Al}_2\text{O}_3$ ,  $\text{MgO}$  and  $\text{ZnO}$ . In each instance the insulators were prepared according to the procedure described in Example 1. Compositions and test results are presented in Table V, below.

ingredient, wherein the minor component is composed of not more than 20 percent by weight of a flux selected from the group consisting of at least one oxide of calcium, strontium and barium, not more than 5 percent by weight of an oxide of boron, not more than 20 percent by weight of a refractory oxide selected from the group

TABLE V

| Body No. | Mol Percent  |                         |              |              | Additives, Grams per 1,000 grams $\text{BeO}$ , $\text{Al}_2\text{O}_3$ , $\text{MgO}$ and $\text{ZnO}$ | Electrical Resistance (Megohms) at 1,350° F. | Thermal Diffusivity, Seconds |         | Dye Test   |
|----------|--------------|-------------------------|--------------|--------------|---------------------------------------------------------------------------------------------------------|----------------------------------------------|------------------------------|---------|------------|
|          | $\text{BeO}$ | $\text{Al}_2\text{O}_3$ | $\text{MgO}$ | $\text{ZnO}$ |                                                                                                         |                                              | Cone 16                      | Cone 31 |            |
| 79       | 47.3         | 16.1                    | 16.1         | 20.4         | (*)                                                                                                     | 25                                           | 14.9                         | 14.40   | Mat. Mat.  |
| 80       | 39.6         | 5.6                     | 35.8         | 19.0         | (*)                                                                                                     | 1                                            | 16.2                         | 16.4    | Mat. Mat.  |
| 81       | 22.9         | 5.8                     | 55.5         | 15.8         | (*)                                                                                                     | 82                                           | 23.3                         | 22.2    | Mat. Mat.  |
| 82       | 58.9         | 10.6                    | 17.1         | 13.3         | (*)                                                                                                     | 100+                                         | 12.5                         | 12.5    | Mat. Mat.  |
| 83       | 43.6         | 11.0                    | 35.1         | 10.2         | (*)                                                                                                     | 100+                                         | 15.6                         | 15.4    | Mat. Mat.  |
| 84       | 62.4         | 15.8                    | 16.7         | 5.0          | (*)                                                                                                     | 100+                                         | 100+                         | 13.0    | U. F. Mat. |

\*Indicates that the additives consisted of 15.5 grams of whiting, 20.7 grams of talc, and 15.5 grams of bentonite per 1,000 grams of  $\text{BeO}$ ,  $\text{Al}_2\text{O}_3$ ,  $\text{MgO}$  and  $\text{ZnO}$ .

It will be noted by reference to Tables I and II, above, that bodies fired from binary mixtures of  $\text{BeO}$  and  $\text{ZnO}$  within the limits claimed herein are particularly advantageous, because they have wide firing ranges, many such bodies being matured when fired either to cone 16 or to cone 31. Specifically, insulators composed predominantly of  $\text{ZnO}$  and  $\text{BeO}$  in ratios of 1 mol of  $\text{ZnO}$  to from 4 to 300 mols of  $\text{BeO}$ , are preferred; most desirably, the ratio is 1 mol of  $\text{ZnO}$  to from 4 to 13 mols of  $\text{BeO}$ . Another group of preferred insulators within this group has a composition of at least 80 mol percent of  $\text{BeO}$  and at least  $\frac{1}{3}$  mol percent of  $\text{ZnO}$ .

It is to be understood that the invention is not limited to the use of pure oxides, as carbonates, hydroxides, and other compounds which yield the oxides upon firing are equally operable. For example,  $\text{Mg}(\text{OH})_2$ ,  $\text{Al}(\text{OH})_3$ ,  $\text{MgCO}_3$ ,  $\text{ZnCO}_3$ , and the like, can be used instead of  $\text{Al}_2\text{O}_3$ ,  $\text{ZnO}$ , and  $\text{MgO}$ . When such compounds are used instead of the oxides, they should be used in proportions such that the fired insulator contains the oxide in the proportions set forth herein.

This application is a continuation in part of application Serial No. 766,648 filed August 6, 1947, now abandoned.

Having described the invention, I claim:

1. A zinc oxide containing sintered ceramic electrical insulator showing by chemical analysis at least 60 per-

50 consisting of titanium, zirconium, cerium and tin, and wherein the sum of the mols of oxides of titanium, zirconium, cerium and tin is not more than half the sum of the mols of alumina and magnesia plus one-twentieth the mols of beryllia.

55 2. A sintered ceramic electrical insulator as claimed in claim 1 in which the composition of the major component is represented by the shaded area of Fig. 1 of the attached drawings.

3. A sintered ceramic insulator as claimed in claim 1 in which the composition of the major component is represented by the shaded area of Fig. 2 of the attached drawings.

60 4. A sintered ceramic electrical insulator as claimed in claim 1 in which the composition of the major component is represented by the shaded portion of Fig. 3 of the attached drawings.

5. A sintered ceramic electrical insulator having a high hot dielectric value and high heat conductivity which is composed as shown by chemical analysis, of at least 60 percent by weight of  $\text{ZnO}$  and  $\text{BeO}$  in ratios of 1 mol of  $\text{ZnO}$  to from 4 to 300 mols of  $\text{BeO}$ .

65 6. A sintered ceramic electrical insulator having exceptionally long firing range which is composed, as shown by chemical analysis, of at least 60 percent by weight of  $\text{ZnO}$  and  $\text{BeO}$  in a ratio of 1 mol of  $\text{ZnO}$  to from 4 to 13 mols of  $\text{BeO}$ .

11

7. A sintered ceramic electrical insulator having a composition by chemical analysis of at least 80 mol percent BeO and at least  $\frac{1}{3}$  mol percent of ZnO.

8. A sintered ceramic electrical insulator having a composition by chemical analysis of at least 20 mol percent of Al<sub>2</sub>O<sub>3</sub> and at least 50 mol percent of ZnO.

9. A sintered ceramic electrical insulator having a high hot dielectric value which is composed predominantly, as shown by chemical analysis, of ZnO and Al<sub>2</sub>O<sub>3</sub> in amounts from 61 $\frac{1}{3}$  mol percent to 71 $\frac{1}{3}$  mol percent 10 and from 38 $\frac{1}{3}$  mol percent to 28 $\frac{1}{3}$  mol percent, respectively.

10. A sintered ceramic electrical insulator having a composition by chemical analysis of at least 60 mol percent of MgO and at least  $\frac{1}{3}$  mol percent of ZnO.

11. A sintered ceramic electrical insulator having a high hot dielectric value which is composed predominantly, as shown by chemical analysis, of ZnO and MgO in amounts from 2.4 mol percent to 12.4 mol percent, and 87.6 mol percent to 97.6 mol percent respectively.

12. A sintered ceramic electrical insulator which consists essentially of at least 60 percent by weight of a major component having a composition represented by the portion of Fig. 7 of the attached drawings lying between a plane through the points 25, 19, 11, and a second plane 25 through the points 25, 14, and 13, and from a trace to 40 percent by weight of a minor component consisting essentially of at least one metal oxide modifying ingredient selected from the group consisting of oxides of calcium, titanium, zirconium, cerium and tin, but not over 30 20 percent by weight of calcium oxide, and not over 20 percent by weight of the four last-named oxides, and

5

10

15

20

25

30

35

12

wherein the sum of the mols of oxides of titanium, zirconium, cerium and tin is not more than half the sum of the mols alumina and magnesia plus one-twentieth the mols of beryllia.

13. A sintered ceramic electrical insulator which consists essentially of at least 60 percent by weight of a major component having a composition represented by the portion of Fig. 8 of the attached drawings lying between a plane through the points 40, 41, 42 and a second plane through the points 44, 45 and 46, and from a trace to 40 percent by weight of a minor component consisting essentially of at least one metal oxide modifying ingredient selected from the group consisting of oxides of calcium, titanium, zirconium, cerium and tin, but not over 20 percent by weight of calcium oxide, and not over 20 percent by weight of the four last-named oxides, and wherein the sum of the mols of oxides of titanium, zirconium, cerium and tin is not more than half the sum of the mols alumina and magnesia plus one-twentieth the mols of beryllia.

#### References Cited in the file of this patent

##### UNITED STATES PATENTS

|           |           |       |               |
|-----------|-----------|-------|---------------|
| 2,033,300 | Reichmann | ----- | Mar. 10, 1936 |
| 2,268,903 | Sawyer    | ----- | Jan. 6, 1942  |
| 2,269,508 | Barton    | ----- | Jan. 13, 1942 |
| 2,336,182 | McDougal  | ----- | Dec. 7, 1943  |

##### FOREIGN PATENTS

|         |         |       |              |
|---------|---------|-------|--------------|
| 7,743   | France  | ----- | 1907         |
| 653,581 | Germany | ----- | Dec. 7, 1943 |